

[54] FLEXIBLE POWER CABLE

[75] Inventors: Theodore E. Hansen; Floyd A. Wilson, both of Marion, Ind.

[73] Assignee: The Anaconda Company, New York, N.Y.

[22] Filed: June 18, 1973

[21] Appl. No.: 371,320

[52] U.S. Cl. 174/113 R, 174/116, 174/120 SR

[51] Int. Cl. H01b 7/02

[58] Field of Search 174/116, 113.R, 120 AR, 174/120 SR, 110 R, 1 PM

[56] References Cited

UNITED STATES PATENTS

2,732,422 1/1956 Rapp..... 174/116 X  
3,710,009 1/1973 Hoeg..... 174/120 AR

OTHER PUBLICATIONS

Avisun Corporation Bulletin, "Gade TD-321D Gen-

eral Purpose Electrical Insulating Polymer," 5-1966. Aamodt et al., "Propylene-Based Copolymers in Wire and Cable Application," 12th Annual Wire and Cable Symposium, 12/63, 29 pages

Rosato "Electrican Wire and Cable Plastics - What Ahead," in Wire & Wire Products, 3/70, pp. 49 and 56.

Jones, "An Oil Extended Ethylene-Propylene Rubber for Cable Insulations and jackets," in Wire 11/66, pp. 1822-1826.

Primary Examiner—E. A. Goldberg

Attorney, Agent, or Firm—Victor F. Volk

[57] ABSTRACT

Power cable such as pendant cable is found to have improved flex life when it combines propylene-ethylene copolymer insulation on the individual conductors with a polyurethane thermoplastic overall jacket.

4 Claims, 1 Drawing Figure



PATENTED DEC 31 1974

3,857,996



## FLEXIBLE POWER CABLE

## BACKGROUND OF THE INVENTION

Flexible electric cables, and particularly cables for use suspended in pendants where they are subjected to repeated folding and unfolding and where interruptions in service due to cable failure are costly and the failures themselves may be dangerous, are the objects of continuing research for means of improving their flex life. Cables in general use today greatly outlive the cables of a decade ago by reason of a number of cable improvements, each of which was the survivor of a number of proposed improvements which did not test out. In one form of flex life test, or fatigue test, these cables are loaded with weights pulled back and forth over sheaves until conductors in the cable break or are short circuited. Clearly, the flex life performance of a proposed cable is unpredictable since, if it were not, such expensive, time-consuming, test programs would not be necessary. The elements of a cable interact in such a complex manner that no adequate theory has ever been developed for the prediction of cable performance and each proposed new cable construction must be extensively tested in the laboratory and in field trials.

## SUMMARY

We have invented an improved flexible cable which, as shall be shown, outlasts presently known constructions due to a synergism of the cable elements as now, for the first time, combined. Our novel, improved flexible power cable comprises, in combination, a plurality of copper conductors, each stranded from a plurality of wires, a heavy wall of propylene-ethylene copolymer insulation covering each of the conductors and a polyurethane thermoplastic jacket surrounding the conductors with their walls of insulation. In a preferred embodiment of our invention, the insulated conductors are helically cabled together to form a flexible core. The polyurethane thermoplastic used for the jacket may advantageously be based on polytetramethylene ether.

## BRIEF DESCRIPTION OF THE DRAWING

The FIGURE shows a section of a cable of our invention.

## DETAILED DESCRIPTION OF PREFERRED EMBODIMENT

In the FIGURE, a cable of our invention, indicated generally by the numeral 10, has four bare soft copper conductors 11-14 each stranded of 65 No. 30 Awg (American wire gage) wires in a bunched left hand lay. The conductors 11-14 are each insulated with an extruded wall 16 of a propylene-ethylene copolymer, 30 mils in thickness. A suitable copolymer for use in the walls 16 is available commercially from the Avison Corp. under their trademark "Olemer" and grade TD-321. The copolymer we have found suitable for insulations in our cable is distinguished from monomeric polypropylene in having a much lower brittle point when tested in accordance with ASTM D-746-57T. The brittle point of a selected insulation 16 is -16C and a copolymer having a brittle point of at most -10C should be used. The copolymer is essentially distinguished from monomeric polyethylene in having higher tensile strength, modulus and melt temperature. The copolymer of the walls 16 exhibits a yield strength of

4,100 pounds per square inch when tested according to ASTM test method D-638-61T, a 100 percent modulus of 1,170 pounds per square inch when tested according to ASTM test method D-412, and a dilatometer melting point of 165C when tested according to ASTM test method D-785-60T. These values should, in any event, exceed 950 pounds per square inch for the 100 percent modulus, 3,700 pounds per square inch for the yield strength, and 155C for the dilatometer melting point.

Each of the conductors 11-14 covered with a layer 16 comprises a strand 17, 18, 19, 20 and the four strands are cabled together with about a three-inch right hand lay. Over the bunched conductors 11-14 and under the walls 16, we have applied a one-half mil longitudinal polyester tape 21. These are applied at the extrusion machine and prevent the extruded composition from penetrating the wire strands. It is known to stabilize the copolymer compositions against a poisoning effect of copper by incorporation of inhibitors such as oxanalide and the composition of walls 16 is so stabilized, but the tapes 21 add further protection against copper migration into the insulation. During the cabling operation, the cable core is rounded out conventionally by the inclusion of paper wrapped rayon fillers 22.

A thirty mil thick jacket 23 of polyurethane thermoplastic has been extruded over the cable strands 17-20. A suitable composition for the jacket 23 is commercially available from Uniroyal, Inc. under their trademark Roylar, designation XE-87-101 which is based on polytetramethylene ether. This composition has the following unaged typical properties:

| ASTM TEST METHOD               |        |      |
|--------------------------------|--------|------|
| Shore A hardness               | D-2240 | 87   |
| Tensile Modulus, psi           | D-412  |      |
| 10%                            |        | 530  |
| 50%                            |        | 940  |
| 100%                           |        | 1170 |
| 300%                           |        | 2340 |
| Ultimate Tensile Strength, psi | D-412  | 5750 |
| % Elongation                   | D-412  | 510  |
| 200% Elongation Set, %         | D-412  | 16   |
| Elongation Set at Break %      | D-412  | 20   |
| Bell Brittle Point, F          | D-746  | 100  |
| Specific Gravity               |        | 1.17 |
| Melt Temperature               |        | 340F |

A 12-foot length of the cable 10 was tensioned at 165 pounds and pulled back and forth over a 6-inch diameter sheave at a rate of 10 cycles per minute. For comparison, the same test was performed on a comparable four conductor, No. 12 Awg, rubber insulated, neoprene jacketed cable. The cable 10 of our invention withstood 4,094 cycles compared to 1,374 cycles for the standard cable before one of the conductors opened.

The foregoing description has been exemplary rather than definitive of our invention for which we desire an award of Letters Patent as defined in the following claims.

We claim:

1. A flexible power cable comprising, in combination,
  - A. a plurality of copper conductors, each being stranded of a plurality of wires,
  - B. a heavy wall of propylene-ethylene copolymer insulation having a yield strength of at least 3,700 pounds per square inch and a dilatometer melting

- point of at least 155°C covering each of said conductors, and  
C. a polyurethane thermoplastic jacket surrounding said conductors having said walls of insulation.  
2. The cable of claim 1, wherein said conductors being covered by said walls, are helically cabled to-

gether to form a flexible core.

3. The cable of claim 1, wherein said polyurethane is based on polytetramethylene ether.  
4. The cable of claim 2, wherein said polyurethane is based on polytetramethylene ether.

\* \* \* \* \*

10

15

20

25

30

35

40

45

50

55

60

65